

# UNITED STATES PATENT OFFICE.

GEORGE H. KEITH, OF SATSOP, WASHINGTON.

## CLEANING AND POLISHING COMPOSITION.

1,146,173.

Specification of Letters Patent. Patented July 13, 1915.

No Drawing.

Application filed March 10, 1914. Serial No. 823,813.

To all whom it may concern:

Be it known that I, GEORGE H. KEITH, a citizen of the United States, residing at Satsop, in the county of Chehalis and State of Washington, have invented a new and useful Cleaning and Polishing Composition, of which the following is a specification.

The invention relates to improvements in cleaning and polishing composition.

- 10 The object of the present invention is to provide a composition designed particularly for use on automobiles and various other vehicles for cleaning and polishing painted or varnished surfaces, and adapted to effect an easy removal of dirt, and apply a thin coating or film of wax to such surfaces for enabling the same to be polished and brightened.

20 The composition consists of the following ingredients, combined in the proportions stated, viz:

Pure beeswax ----- 5 drams.  
Gasolene ----- 1 quart.

- 25 The beeswax is allowed to dissolve in the gasolene for a period of about a week, and the mixture should be well shaken. This is sufficient to cause the beeswax to become thoroughly dissolved, and the cleaning and polishing composition, which is in the form of a liquid, is applied by means of a sponge or the like, to the painted, varnished, or other surface to be cleaned and polished. The gasolene of the cleaning and polishing composition quickly evaporates from the surface to which the same is applied, acting

as a cleaning element in removing dirt from the surface, and leaving the surface coated with a thin film of beeswax. The thin film or coating of beeswax operates as a polishing agent, and the coated surface is rubbed down and polished with a soft cloth. The cleaning and polishing fluid, when applied to a painted or varnished surface in this manner, results in a highly polished surface, which is free from dirt.

40 What is claimed is:

1. The herein described liquid composition for cleaning and polishing painted and varnished surfaces consisting of gasolene and beeswax combined in substantially the proportions stated, the beeswax being completely dissolved in the gasolene in sufficient quantity to leave a thin polishing film or coating on the surface to which the liquid composition is applied, and the gasolene operating as a cleaning agent.

2. The herein described liquid composition for cleaning and polishing painted and varnished surfaces consisting of gasolene, one quart, and beeswax, five drams, dissolved in the gasolene so that when the composition is applied to such a surface, the gasolene will evaporate and leave a thin film or coating of wax on the said surface.

60 In testimony, that I claim the foregoing as my own, I have hereto affixed my signature in the presence of two witnesses.

GEORGE H. KEITH.

Witnesses:

CIRAS. H. RAMEY,  
ORTON GLENN.